

## UNITED STATES PATENT OFFICE

2,247,046

## EXTREME PRESSURE LUBRICANT

Henry G. Berger and Darwin E. Badertscher,  
Woodbury, and Francis M. Seger, Pitman, N. J.,  
assignors to Socony-Vacuum Oil Company, In-  
corporated, New York, N. Y., a corporation of  
New York

No Drawing. Application October 23, 1940,  
Serial No. 362,373

9 Claims. (Cl. 252—48)

This invention, which is a continuation in part of that disclosed in our copending application Serial No. 177,891, filed December 3, 1937, has to do in a general way with the art of lubrication and is more particularly concerned with the development of a lubricant composition adapted for use under extreme pressure conditions.

As is well known to those familiar with the art, the ordinary type of hydrocarbon lubricant, comprised only of a petroleum fraction, is incapable of withstanding the enormous pressures encountered between engaged surfaces in various types of modern machinery, such as the hypoid gears used in motor vehicles. This fact has led to the development of the so-called extreme pressure lubricant, which is comprised of a suitable carrying agent, such as mineral oil, containing a minor proportion of an ingredient which under the extreme pressure conditions encountered will provide or form between the engaged surfaces a lubricating film capable of withstanding these high pressures. Ingredients of the type just referred to are known as extreme pressure ingredients or extreme pressure (E. P.) bases, and numerous materials have been proposed for such use. Among the various E. P. bases which have been proposed and which have met with varying degrees of success are organic materials which contain sulfur and chlorine. Our present invention is related to this general type of compound.

It is a primary object of this invention to provide an extreme pressure lubricant which contains a new and novel sulfur-and-chlorine-containing material or compound capable of giving extreme pressure lubricant properties to a carrying agent such as a hydrocarbon lubricant oil otherwise incapable of withstanding these extreme pressure conditions. In this regard, we have discovered that the class or group of compounds or reaction products obtained by reacting various reactive organic compounds with perchloromethylmercaptan are very effective extreme pressure lubricant addition agents. These materials have the advantage of being cheap and easily prepared. Perchloromethylmercaptan itself and its low molecular weight derivatives are very effective E. P. bases, but we prefer to use the higher molecular weight derivatives because

they are more desirable from the standpoint of odor.

The perchloromethylmercaptan derivatives which we have found to be particularly useful as E. P. bases may be broadly divided into two general classifications: namely, (1) products obtained by reacting perchloromethylmercaptan with organic compounds containing an active hydrogen or an active metal atom, or both; and (2) products obtained by reacting perchloromethylmercaptan with unsaturated organic materials such as animal and vegetable oils, cracked petroleum stocks, etc. Reaction products of the type encompassed by class (2) above were made the subject of our application Serial No. 177,890, filed December 3, 1937.

Our aforesaid application Serial No. 177,891, of which the present application is a continuation in part, was broadly directed to reaction products of group (1), wherein the secondary reactant is an organic compound containing an active hydrogen atom or an active metal atom, or both. This broad subject matter has now been embodied in another continuation in part of Serial No. 177,891: namely, application Serial No. 362,372 filed concurrently herewith.

The present invention is concerned with a group of perchloromethylmercaptan reaction products falling into the broad class designated above as group (1). More specifically, the present invention contemplates extreme pressure bases which are obtained by reacting perchloromethylmercaptan with organic compounds having the general formula  $RSX$ , in which R represents a hydrocarbon radical selected from the group consisting of alykyl, aryl, aralkyl, and alkaryl radiacals and X represents hydrogen or the hydrogen equivalent of a metal. Compounds falling under this general formula include the mercaptans with their corresponding mercaptides, the thiophenols with their corresponding thiophenates, etc. Typical specific compounds are propyl mercaptan; sodium propyl mercaptide; potassium propyl mercaptide; butyl mercaptan; sodium butyl mercaptide; potassium butyl mercaptide; amyl mercaptan; sodium amyl mercaptide; potassium amyl mercaptide; hexyl mercaptan; sodium hexyl mercaptan; potassium hexyl mercaptan; thiophenol; sodium thiophenate, etc.

Perchloromethylmercaptan, the primary reactant used in synthesizing the reaction products contemplated herein, is a chlorinated substituted sulfur chloride having the formula  $\text{Cl}_3\text{C}-\text{SCl}$ . It can be prepared by the chlorination of carbon disulfide according to the method of Helfrich and Reid (Journ. Amer. Chem. Soc. 43, 591 (1921)). For example, carbon disulfide containing about .4 per cent by weight of iodine was chlorinated in the absence of direct sunlight at a temperature maintained below 25° C. until the volume of the reaction mixture had doubled. This crude reaction product, which contains carbon tetrachloride and sulfur chlorides in addition to perchloromethylmercaptan, can be used in the preparation of the reaction products contemplated by this invention, but it is preferable to purify the crude product by distillation on a water bath at 100° C. followed by steam distillation. Subsequent vacuum distillation of the material refined in this manner indicated that the steam-distilled material was practically pure.

The general procedure for preparing reaction products of the type contemplated herein may be obtained from the following illustrative examples.

#### EXAMPLE ONE

##### Reaction of perchloromethylmercaptan with amyl mercaptan

Perchloromethylmercaptan was treated with an equimolar amount of amyl mercaptan. The reaction was exothermic and was accompanied by the evolution of hydrogen chloride. The slight excess of perchloromethylmercaptan in the reaction product was removed (steamed out) and the product was dried by filtration. This product contained 22.1 per cent sulfur and 38.1 per cent chlorine.

#### EXAMPLE Two

##### Reaction of perchloromethylmercaptan with potassium amyl mercaptide

Potassium amyl mercaptide was prepared by shaking 21 grams (0.2 mole) of amyl mercaptan with an equivalent amount of KOH in water. The somewhat turbid solution was added to 37 grams (0.2 mole) of perchloromethylmercaptan in 100 cc. of petroleum ether, and the two solutions were stirred together for one hour at room temperature. There was an initial temperature rise of 5° C., and a water bath was used to prevent further heating. The petroleum ether solution was then water-washed and the ether distilled off, leaving 45 grams of product which was an oil. This product on distillation yielded a fraction boiling at about 77° C. at 1 mm. which contained 25.6% sulfur and 33.2% chlorine.

To demonstrate the effectiveness of the reaction products contemplated by this invention as extreme pressure lubricant ingredients, we have prepared and tested lubricant compositions comprised of mineral oil and typical reaction products of the class disclosed herein. More specifically, we have prepared blends of the reaction products of the foregoing examples in a mineral oil having a Saybolt Universal viscosity of 80-90 seconds at 210° F. and have subjected samples of such lubricant blends to the Almen pin test, described by Wolf and Mougey, Proc. A. P. I., 1932, pages 118-130, and the S. A. E. test, described in S. A. E. Journal 39, 23-4 (1936). These two tests are commonly accepted in the art as standards to determine the extreme pressure characteristics of a lubricant. In Table I below, we show the results obtained with such tests, 75

using the oil without the addition agent and samples of the same oil blended with perchloromethylmercaptan derivatives of the type contemplated by this invention.

5

TABLE I

| Reaction product added                                    | Percent | Extreme pressure tests (lbs. failed) |                                                                           |
|-----------------------------------------------------------|---------|--------------------------------------|---------------------------------------------------------------------------|
|                                                           |         | Almen                                | S. A. E. (755 R. P. M. 14:6:1 rubbing ratio; 8.35 lbs./sec. loading rate) |
| None                                                      |         | 3,000                                | 40-70                                                                     |
| $\text{Cl}_3\text{CSCl}+\text{amyl mercaptan}$            | 5       | 30,000                               | 580+                                                                      |
| $\text{Cl}_3\text{CSCl}+\text{potassium amyl mercaptide}$ | 3       | 29,000                               | 310*                                                                      |
| $\text{Cl}_3\text{CSCl}+\text{tertiary butyl mercaptan}$  | 3       | 30,000                               | 360*                                                                      |

\*These values were obtained at 1,000 R. P. M. instead of 755. The blank oil failed in the S. A. E. test at 1,000 R. P. M. at a load of 20 lb.

From the foregoing examples it will be seen that the perchloromethylmercaptan condensation products contemplated by this invention are highly effective extreme pressure lubricant bases. The amount of these materials used may vary from about .5 per cent to about 20 per cent, but in general the lower percentages ranging from 5 per cent to 10 per cent are preferred.

Although we have indicated in the foregoing description that a mineral lubricating oil is a preferred carrying agent for the extreme pressure agent, it is not our intention that the invention be limited in this regard. The invention includes broadly extreme pressure lubricants containing perchloromethylmercaptan condensation products of the aforesaid type dissolved, dispersed or emulsified in any suitable carrying medium such, for example, as fatty vegetable and animal oils; light petroleum hydrocarbons such as kerosene; benzene and related hydrocarbons; alcohols; esters, ethers, etc.

It is to be understood that while we have herein described and illustrated the invention with certain specific examples, the invention is not limited to the specific examples given but includes within its scope such changes and modifications as fairly come within the spirit of the appended claims.

We claim:

1. An extreme pressure lubricant comprising a hydrocarbon oil and in admixture therewith a minor proportion of the product obtained by the reaction of perchloromethylmercaptan with a compound having the general formula  $\text{RSX}$ , wherein  $\text{R}$  represents a radical selected from the group consisting of alkyl, aryl, aralkyl, and alkaryl radicals and  $\text{X}$  represents an element selected from the group consisting of hydrogen and metal, the said reaction product containing both sulfur and chlorine and being present in the oil in an amount sufficient to increase its load-carrying capacity.

2. An extreme pressure lubricant comprising a hydrocarbon lubricant oil and in admixture therewith a minor proportion of the product obtained by the reaction of perchloromethylmercaptan with a mercaptan, said product containing both sulfur and chlorine.

3. An extreme pressure lubricant comprising: a hydrocarbon lubricant oil and in admixture therewith a minor proportion of the product obtained by the reaction of perchloromethylmer-

captan with a mercaptide, said product containing both sulfur and chlorine.

4. An extreme pressure lubricant comprising: a hydrocarbon lubricant oil and in admixture therewith a minor proportion of the product obtained by the reaction of perchloromethylmercaptan with an amyl mercaptan, said product containing both sulfur and chlorine.

5. An extreme pressure lubricant comprising: a hydrocarbon lubricant oil and in admixture therewith a minor proportion of the product obtained by the reaction of perchloromethylmercaptan with potassium amyl mercaptide, said product containing both sulfur and chlorine.

6. An extreme pressure lubricant comprising: a hydrocarbon lubricant oil and in admixture therewith a minor proportion of the product obtained by the reaction of perchloromethylmercaptan with a tertiary butyl mercaptan, said product containing both sulfur and chlorine.

7. An extreme pressure lubricant composition comprising: a minor proportion of the chlorine-and-sulfur-containing product obtained by the reaction of perchloromethylmercaptan with a compound having the general formula  $RSX$ , 25 wherein R is selected from the group consisting of alkyl, aryl, aralkyl and alkaryl radicals and

X represents hydrogen or the hydrogen equivalent of a metal; and a major proportion of a carrying medium, which composition, when applied to metallic bearing surfaces, will form a lubricant film capable of withstanding extreme pressure conditions.

8. An extreme pressure lubricant composition comprising a minor proportion of the chlorine-and-sulfur-containing product obtained by the reaction of perchloromethylmercaptan with a mercaptan, in admixture with a major proportion of carrying medium, which composition, when applied to metallic bearing surfaces, will form a lubricant film capable of withstanding extreme pressure conditions.

9. An extreme pressure lubricant composition comprising a minor proportion of the chlorine-and-sulfur-containing product obtained by the reaction of perchloromethylmercaptan with a mercaptide, in admixture with a major proportion of carrying medium, which composition, when applied to metallic bearing surfaces, will form a lubricant film capable of withstanding extreme pressure conditions.

HENRY G. BERGER.  
DARWIN E. BADERTSCHER.  
FRANCIS M. SEGER.